

May 6, 1941.

H. NIPPER

2,241,270

PROCESS FOR WORKING IRON CARBON ALLOYS

Original Filed Nov. 8, 1933 2 Sheets-Sheet 1

Fig. 1



Fig. 2



Fig. 3



Fig. 4



INVENTOR

*Heinrich Nipper*

BY

*McLanna, Hintercorn & Morebach*

ATTORNEYS

May 6, 1941.

H. NIPPER

2,241,270

PROCESS FOR WORKING IRON CARBON ALLOYS

Original Filed Nov. 8, 1933 2 Sheets-Sheet 2

Fig. 5



Fig. 6



Fig. 7



Fig. 8



INVENTOR

*Heinrich Nipper*

BY

*McLanna, Wintercorn & Grubach*

ATTORNEYS

## UNITED STATES PATENT OFFICE

2,241,270

## PROCESS FOR WORKING IRON CARBON ALLOYS

Heinrich Nipper, Aachen, Germany, assignor to The Timken Roller Bearing Company, Canton, Ohio, a corporation of Ohio; Gunite Foundries Corporation, Rockford, Ill., a corporation of Illinois, and Stellum, Inc., Cleveland, Ohio, a corporation of Ohio

Original application November 8, 1933, Serial No. 697,138. Divided and this application August 6, 1938, Serial No. 223,465. In Germany November 8, 1932

4 Claims. (Cl. 29—148)

Pig iron, grey and white cast iron, and malleable iron have hitherto been regarded as being unworkable, either cold or hot. Since, in the case of steel, it has been customary to reduce the rolling temperature with increase of the carbon content one reason for the failure to roll cast iron will presumably have to be attributed to a far too low temperature being employed.

Comprehensive experiments of the inventor have shown that pig iron, grey and white cast iron and malleable iron are readily workable, for example by rolling, pressing, forging, hammering or drawing, etc., if, depending on the composition of the material, temperatures, which, in respect to the heat treatment of cast iron, are unusually high, for example from 950 up to about 1150° C. and above, are maintained.

In working up the material, cast ingots, billets or plates of varying thickness, are heated uniformly to rolling temperature in heating furnaces and then rolled in rolling mills. The reduction in cross-section, which on the average may amount to about 20% per pass, as well as the frequency of reheating, varies with the thickness of the rolled plates and profiles. The small degree of brittleness of the side edges, which under certain circumstances may occur owing to too much cooling, may be entirely avoided by rolling the material in the last passes between heavy plates. By doing so excessive cooling is eliminated and rolling to smaller gauges is made possible. The same result is obtained by doubling or by simultaneously rolling out a great number of thin plates. In the case of very thin plates it is advisable to roll out the material between thin steel plates. In this case a high carbon content of the steel plates is desirable, in order to avoid diffusion. If compound material, which is a product made by simultaneously rolling and welding cast iron plates and steel plates, is to be produced the starting material may consist of cast iron plates, which are covered with steel plates and are welded to the steel plates at the edges before they are charged into the heating furnace. By this or any other suitable manner, the contacting surfaces of the material are protected against the influence of the furnace gases. It is further possible in the rolling to thus produce, by welding and diffusion of the carbon from the cast iron into the soft steel material, a plate consisting half and half of cast iron and steel, or, alternatively, two steel plates with a core of cast iron or, also, a core of steel with two coverings of cast iron. The cast iron and steel ad-

here firmly together and cannot be separated from one another.

Figures 1 and 2 show the compound material which has been so produced, at a magnification of 100 and 250 respectively. Figure 3 shows a normal cast iron, containing about 2% silicon and 3% carbon, rolled out and cooled in air, at a magnification of 250. Figure 4 shows a cast iron with a high content of carbon, containing about 3.8% C and about 2.4% Si, after rolling and heating, at a magnification of 250. Figure 5 shows a white cast iron, low in silicon, containing about 3.2% C and 0.5% Si, after rolling and cooling in air, at a magnification of 250. Figure 6 shows a low carbon and high silicon containing iron after rolling and subsequent annealing at a low temperature to produce a ferritic matrix. Figure 7 shows a material, which was rolled in the white initial state and annealed after rolling to produce a ferritic matrix. Figure 8 shows a material, which was rolled in the white initial state and after rolling was freed from carbon by heating in agents, which produce oxidizing gases, and was thus obtained in the ferritic state.

All the figures show that graphite, temper carbon and also Ledeburite can be stretched to fibres in the direction of rolling. The materials produced have considerable strength and can also be joined with one another satisfactorily by soldering and welding, such as butt-welding. In the rolled cast irons the tensile strength was 67 kgms./mm.<sup>2</sup> before annealing and 54 kgms./mm.<sup>2</sup> after annealing. The rolled malleable iron showed a tensile strength of from 110 up to 120 kgms./mm.<sup>2</sup> with 5% elongation in the unannealed state. After annealing the same material showed a tensile strength of 50-60 kgms./mm.<sup>2</sup> with an elongation of 15-20%.

40 This is a division of my copending application, Serial No. 697,138, filed November 8, 1933.

The essential advantage of cast iron is that it can be easily melted and cast. In the case of sub-eutectic iron, the capability of being cast increases with the increase in carbon content. The capability of being rolled, however, gradually decreases as the content of highly carbon components, such as ledeburite, graphite and temper carbon, increases. It follows from this that for the production of rolled cast iron plates, an alloy is most desirable which does not have too high a content of high carbon components to permit rolling, but has a sufficient content of such components to permit satisfactory melting and casting. Accordingly, in the case of normal

unalloyed cast iron, which has been cast without special precautions as to solidification (chill mold, quenching, etc.) in normal sand (refractory) molds, the carbon content should be below about 3%. Cast iron alloys having a low content of carbon can be rolled more easily, but are more difficult to cast. This, as well as the slight tendency to become graphitized in the cast or rolled state may be compensated by a high content of silicon or other elements.

The cast material may have various structures. With martensitic, troostitic, sorbitic, pearlitic or ferritic matrix, it may contain high carbon components such as cementite, ledeburite, graphite or temper carbon, in a more or less finely distributed, non-uniform or uniform arrangement. These high carbon components, dispersed in the matrix, can be given definite preferably fibrous form by the rolling operation. It is, however, also possible, by subjecting an originally white cast iron or non-annealed malleable iron to heat treatment after the rolling only, to produce a normal stable or unstable temper carbon formation in any desired matrix. Steels containing free carbon in the form of graphite or temper carbon were never produced consistently, so that a systematic production of graphitic line structure even of as little as a few tenths of one per cent of free carbon is in itself an important feature of the present invention. White cast iron can be readily rolled at a suitable temperature, and by subsequent treatment, plain malleabilizing, or annealing in decarburizing agents, it is possible to produce black heart or European (white heart) malleable iron.

The material produced in this manner finds application for many purposes. Piston rings may be produced from sheets containing well-precipitated graphite by the method of stamping or by cutting off sections of a sheet which has previously been bent to tubular shape.

High quality piston rings are today manufactured by casting them individually in very accurate sand molds with a small allowance for machining. Since the small piston rings have only a small cross-section, it is necessary to allow but slight deviation with regard to chemical composition of the material as well as with regard to the manner of melting and casting. Only in this manner is it possible to manufacture piston rings which show a very uniform sorbitic matrix and a uniform distribution of graphite. The composition of the material and the structure of the piston rings have hitherto been governed by the dimensions of the piston rings. In the manufacture of cast piston rings, the yield is only approximately 35-40%, the rest being gates and risers. Today, it is difficult to produce cast piston rings with high elasticity, such as desired for piston rings for motors and compressors operating with high gas pressures.

In manufacturing piston rings in accordance with the present invention, a high quality cast iron of a composition particularly suitable for the purpose is melted in any suitable furnace and cast in a sand or a permanent mold into moderately thin plates of suitable length. After cooling or while still hot from the casting operation, this plate is charged into a reheating furnace and then rolled out to the desired reduced thickness. The rolling process is advantageously started at temperatures between about 1000° and 1150° C.

The number of passes depends on the degree to which the material may be elongated from

one pass to the next, which, in turn, is dependent upon the composition of the material. When cooled down during rolling to a temperature of about 900° C., it is advisable to reheat the material.

The material has high wearing qualities and shows high elasticity. It shows a very dense structure, since it possesses a sorbitic-troostitic, fine grained matrix, and graphite flakes finely distributed at right angles to the rolling plane or parallel thereto. If the material is to be employed for special purposes, any desired hardness can be imparted to it by subsequent heat treatment. The yield in the rolling process is high and the material can easily be cut on the shearing machine.

The manufacture of the finished ring from the sheets made by rolling can be accomplished in different ways:

20 1. An iron plate produced by rolling, of the width of the circumference of the piston ring is bent up to a tube and the individual piston rings are cut off from this tube.

25 2. Strips of the final dimensions of the piston ring are cut out from the iron plate produced by rolling and then bent individually into the proper form.

30 3. Rings having the final dimensions and final form are produced by stamping from an iron plate produced by rolling.

35 In this manner, piston rings of any desired dimensions and of high elasticity can be produced. Moreover, it is possible to impart to the material of these rings any desired matrix, any content of carbon and any desired distribution thereof.

The piston rings may also be manufactured from the compound material consisting of cast iron and steel, which has already been described. It is advantageous, in making the compound material for such rings, to unite the cast iron and steel in such a way that the cast iron in the finished ring will face the cylinder wall. The steel, in such case, may be a normal or special steel, possessing highly elastic properties, causing the piston ring to lie closely against the cylinder wall.

The invention also contemplates the manufacture of bushings and sleeves for contact with moving parts such as the sleeves in the cylinder block of motors and engines, these parts being closely analogous to piston rings and manufactured in the manner heretofore set forth with respect to piston rings. The method permits of the manufacture of these objects of improved characteristics due to the presence of graphite in the metal and the direction of the graphite grain produced in the rolling of the metal.

The materials produced according to the invention are further suitable for brake drums and brake drum inserts subjected to great stresses.

Particularly brake drums and brake drum inserts can advantageously be made from the rolled graphite-containing material with a suitable matrix. For the same purpose, compound-rolled material, cast iron-steel, may also be employed.

Brake drums, which have been made from a normal or special malleable iron, are necessarily very limited with regard to composition, and it is exceedingly difficult to manufacture them so that they comply with all requirements. It is also difficult to always obtain with certainty the desired structure of the iron, or a structure closely resembling the same. If, however, brake drums made from steel are provided with a lining of cast iron, the brake drums become too heavy. This is

the reason why a process for the manufacture of brake drums was introduced, consisting of cast iron being cast in accordance with scientific principles against moderately thin steel brake drums which are of special shape. These brake drums are of a very high quality, the thickness of the cast iron lining depending upon the necessary heat diffusion during the casting process. On the other hand, this method of making brake drums is exceedingly expensive.

The manufacture of the drums is in this case accomplished in the following manner. Steel and cast iron of particularly suitable composition are cast simultaneously in the same mold. A composite material of the desired shape can also be made by casting steel about a cast iron core, or by casting cast iron into a steel sheath and thereafter rolling the material. The material can further be made by rolling plates of cast iron and steel together into strips of the desired shape, welding during the rolling. In all cases the material can be shaped according to the cross-section of one or more brake drums. The strips are cut to the desired length, i. e. to a length corresponding to the circumference of the drum, and are then bent up in the cold or hot state to rings and welded.

The brake drums, which are made according to the foregoing process, show the following advantages:

1. Since cast iron and steel are rolled simultaneously with one another, the materials are completely welded with one another and show an intimate joint. For this reason the brake drums produced are of high safety and low weight.

2. The process enables the best steel and the best cast iron composition to be employed for these special brake drums or shoes, the process being entirely different from those in which these brake drums are made by casting. In this process the composition of the material is not limited to the extent necessary in the manufacture of brake drums by casting.

3. Any desired shape and any desired cross-section of the material can easily be obtained with the aid of the rolling process.

Due to the satisfactory frictional properties of cast materials, in particular cast iron, slide ways and other members, which in use are subjected to frictional stresses, are advantageously made in accordance with the invention from cast materials. For this purpose, certain analyses, for example, iron-carbon alloys, with or without additions of nickel, chromium, molybdenum, vanadium, etc., and certain types of structures, for example, pearlitic, etc., are particularly desirable.

These slide ways and other members are first cast in suitable form, but are not employed in such form, but rolled after casting or subjected to a drawing process or otherwise hot or cold worked, and in this way, brought into the form in which they are employed, after suitable surface or other treatment.

In order to produce the desired structure in the finished product, for example, a predominating pearlitic, sorbitic, martensitic or other suitable structure, it may be advantageous arbitrarily to control the cooling of the piece, which may be still warm from the rolling or be again specially heated, for example, artificially, to retard or to accelerate the cooling. This may be accomplished by bringing the piece into suitably heated rooms (e. g. furnaces), by embedding the same in suitable substances which are good or

bad conductors of heat, (e. g. powder), or bringing the same into liquids, by quenching with the aid of spraying or in any other suitable manner.

The shaping of the slide ways is thus not obtained by casting in accordance with the desired pattern, but by rolling or subsequent working of a cast piece in a heated condition, appropriate quality of structure being imparted to the piece by a suitable treatment.

10 The processes herein described may also be advantageously employed for the production of transformer plates, bearings, checkered or corrugated plates, girders and other structural shapes, grate bars, frame or casing parts for various machines and apparatus, springs, enamelling plates, material to be machined, cutting chisels, etc.

20 The term welding used in this specification in connection with the production of compound material is meant to cover all processes, which render it possible to unite the materials to be fused together in such a way that a permanent cohesion and a safe adhesion is obtained, which is able to resist the mechanical stresses, tending to separate the plurality of materials. Rarely, the separation itself will take place at the boundary line of the two different materials. Normally one of the materials will rather be destroyed if separation is attempted. This is in

30 particular the case in the combination of cast iron and steel. If welding has been effected satisfactorily a considerable diffusion of carbon from the cast iron into the steel takes place, whereby the adhesion of the two materials is so strong that if separation is attempted by force the cast iron breaks in itself, the separating surface being not exposed at all.

35 While I have thus explained the principles and have described and illustrated the preferred 40 manner of utilizing my invention, I am aware that the invention may be otherwise practiced, and I do not wish to be limited except as required by the prior art and the scope of the appended claims.

45 I claim:

1. Improvements in the process for working gray cast iron containing more than 1.5% carbon, comprising heating the alloy to 950° to 50 1150° C. and above, and hot rolling the said alloy in this state.

55 2. The method comprising casting a plate of grey cast iron containing in the region of 3% carbon, heating said plate to a temperature in the region of 1150° C., thereafter hot-rolling the metal and reheating the metal whenever the temperature drops below about 900° C. during the rolling to produce rolled shapes of metal containing graphite carbon.

60 3. The method of making composite products 60 of steel and gray cast iron which comprises casting one of said metals in the molten state against the other in a solid state heating the composite stock to a temperature between about 950° and 1150° C., and hot rolling the stock to the desired 65 shape.

65 4. The method of making composite products 70 of steel and cast iron which comprises casting gray cast iron in molten state against steel in a solid state to form an ingot comprising layers of said metals heating the composite stock to a temperature between about 950° and 1150° C. and hot rolling the stock to the desired shape.

HEINRICH NIPPER.

CERTIFICATE OF CORRECTION.

Patent No. 2,241,270.

May 6, 1941.

HEINRICH NIPPER.

It is hereby certified that error appears in the printed specification of the above numbered patent requiring correction as follows: Page 3, second column, line 58, claim 2, for the word "graphite" read --graphitic--; and that the said Letters Patent should be read with this correction therein that the same may conform to the record of the case in the Patent Office.

Signed and sealed this 8th day of July, A. D. 1941.

(Seal)

Henry Van Arsdale,  
Acting Commissioner of Patents.